

## 1

3,490,909

## SPONTANEOUSLY DEVELOPABLE PHOTO-SOLUBLE SILVER HALIDE DISPERSIONS AND ELEMENTS

Ralph Kingsley Blake, Westfield, N.J., assignor to E. I. du Pont de Nemours and Company, Wilmington, Del., a corporation of Delaware

No Drawing. Continuation-in-part of application Ser. No. 377,122, June 22, 1964. This application Apr. 10, 1967, Ser. No. 629,426

Int. Cl. G03c 1/02, 5/24

U.S. Cl. 96—94

13 Claims

## ABSTRACT OF THE DISCLOSURE

Photosoluble silver halide dispersion layers comprising, before imagewise exposure to light, silver halide crystals that are (1) "spontaneously developable" and (2) have associated therewith, in substantially greater than fog-inhibiting amounts, a silver salt of a 2-mercapto-4-oxazole, thiazole or iminazole having a 4 to 8-membered hydrocarbon nucleus linked to the 4 and/or 5-carbon atom of the azole nucleus, the silver salt being of lower solubility in water than silver chloride and the associated silver halide crystals being less soluble in 10% sodium thiosulfate than untreated crystals, and processes of exposing and processing same. The new photosoluble elements form visible silver halide images which may be intensified by reduction to silver in a conventional nonfogging developer without immediate light fogging prior to intensification.

This application is a continuation-in-part of my co-pending application Ser. No. 377,122 filed June 22, 1964 and entitled Emulsion Layer and Elements, now abandoned.

## BACKGROUND OF THE INVENTION

## Field of the invention

This invention relates to photosoluble (or photosolubilizable) silver halide layers and elements containing the same wherein the layers are "spontaneously developable" being made by prefogging the treated silver halide crystals with radiation and/or by means of chemicals.

## Description of the prior art

There are a number of recently granted U.S. patents on photosoluble layers and elements and processes of image formation using them. Among these patents are 3,155,506-7, 3,155,514-9 (all patented Nov. 3, 1964), the two believed to be most pertinent to the present invention being 3,155,507 and 3,155,519.

Blake 3,155,507 relates to a process which comprises in the order stated, the steps of (a) exposing, imagewise, to actinic radiation a photosoluble silver halide layer containing silver halide crystals made relatively less soluble in a silver halide solvent (e.g., sodium thiosulfate) by treatment with an organic compound capable of forming a silver salt and whose silver salt is less soluble in water than silver chloride, and (b) prior to any reducing step, treating the element with an aqueous solution of a silver halide solvent, thereby effecting solubilization of the silver halide in more exposed areas at a rate substantially greater than in less exposed areas until a positive image comprised of silver halide is produced. Subsequently the silver halide image can be intensified, e.g., by reduction to a silver image.

Blake 3,155,519 relates to photographic silver halide layers of the type described in the previous paragraph but one where the silver salt is a silver mercaptide of a 2-mercaptothiazole having a hydrocarbon nucleus of 4-12

## 2

carbon atoms, preferably phenyl. Blake 3,155,519 claims photographic elements having layers of silver halide crystals previously made to have a lowered rate of solution in a silver halide solvent by treatment with an organic compound capable of forming a silver salt of lower solubility in water than silver chloride. Such elements are capable of yielding positive photographic images of silver halide by exposing them, imagewise, to actinic radiation and then treating in a solution of a silver halide solvent to remove silver halide in the exposed areas. This positive silver halide image can subsequently be intensified by various means, e.g., by reducing the silver halide image to a metallic silver image. The non-optically sensitized elements disclosed above are sensitive only to the shorter end of the visible spectrum, i.e., they cannot be exposed by red, orange, or yellow light and have very little sensitivity to green light.

In U.S. Patent 3,155,519 and the other patents of assignee dealing with photosoluble layers and processes of image formation using such layers, there is no mention made of "spontaneously developable" crystals or layers, or deliberate prefogging by irradiation and/or by means of chemicals.

## SUMMARY OF THE INVENTION

The photosoluble silver halide layers and elements of this invention comprise photosoluble silver halide crystals that are spontaneously developable and have associated therewith in substantially greater than fog-inhibiting amounts a silver salt of a 2-mercapto-4-oxazole, thiazole or iminazole having a 4 to 8-membered hydrocarbon nucleus linked to a 4 and/or 5-carbon atom of the azole nucleus.

## DESCRIPTION OF THE PREFERRED EMBODIMENTS

The photographic layers and elements, e.g., films, plates and papers of this invention comprise, before exposure to actinic light, silver halide crystals that are (1) "spontaneously developable," and (2) have associated therewith in substantially greater than fog inhibiting amounts a silver salt of an azole compound of the formula



where X is a member selected from the group consisting of S, O and NH, R<sub>4</sub> is a hydrocarbon nucleus of 5-8 carbon atoms, e.g., amyl, cyclohexyl, phenyl, and p-methoxyphenyl, and R<sub>5</sub> is a member selected from the group consisting of H and a hydrocarbon nucleus of 5-8 carbon atoms, i.e., the same nuclei as for R<sub>4</sub>.

These silver salts are of lower solubility in water than silver chloride, the silver halide crystals so associated with the silver salt being less soluble in 10% aqueous sodium thiosulfate than untreated silver halide crystals at a predetermined pH and the associated organic compound being present in such an amount, in terms of the ratio of its weight to the surface area of said silver halide crystals, that when admixed in such ratio with an aqueous silver chlorobromide (70/30 mole percent) gelatin emulsion containing 10 g. of gelatin per mole Ag and .57 mg. of Ag per ml., and said silver chlorobromide dispersion is treated with 10%, by weight, aqueous sodium thiosulfate (so that the resulting mixture contains 0.29 mg. of silver and 100 mg. of sodium thiosulfate), at least three times the amount of silver chlorobromide remains undissolved as compared with a similar dispersion successively treated with 5%, by weight, aqueous sodium hypochlorite and 10%, by weight, aqueous sodium thiosulfate (so that the resulting mixture contains 0.29 mg. of silver, 25 mg. of

sodium hypochlorite and 100 mg. of sodium thiosulfate), after vigorous and essentially equal agitation of both dispersions for 30 seconds at 25° C. In the preferred layers and elements, any heavy metal salts present are noble metal salts.

The "spontaneously developable" silver halide crystals can be readily made by prefogging them with radiation and/or by chemicals. In Example V, quantitative tests are disclosed in "Sequence c" which involve processing steps labeled "Fix and Wash" followed by intensification by treatment for 3 minutes at 68° F. with conventional agitation in a specified photographic developer solution labeled "Developer A," followed in turn by a "Final Fix." Silver halide crystals suitable in the present invention should be "spontaneously developable" (i.e., developable without further treatment by radiation or by chemicals) to the extent that over 25% by weight of the silver of said crystals remains as reduced (metallic) silver after being processed according to "Sequence c."

In a practical embodiment of the invention, a gelatino-silver halide photographic emulsion is coated on a suitable support, and the coated element is bathed in a solution of a compound of Formula I which forms a silver salt in intimate association with the silver halide crystals of the photographic emulsion. In a more preferred manner, elements can be prepared by adding the organic compound to the photographic emulsion prior to coating, as also disclosed in Blake U.S. Patent 3,155,519. In either event, the coated element comprises silver halide crystals in intimate association with the said silver salt of the organic compound. The element is photographically fogged either by uniform exposure to actinic radiation or preferably by uniform chemical fogging. Either of these means of fogging the photographic element may occur during the preparation of the element, either before or after (but preferably before) the introduction of the organic compound which forms the silver salt in intimate association with the silver halide crystals. The fogged element thus prepared is capable of forming a positive, photographic image by imagewise exposure to actinic radiation followed by treatment with a silver halide solvent which removes silver halide more rapidly from the exposed than from the unexposed areas. The sensitivity of the element of this invention has been extended by the fogging action so that a positive image can be produced by exposure to long wave length visible light.

The positive silver halide image obtained after treatment with a silver halide solvent may, with or without a water-washing step, be dried and used without further treatment, e.g., for viewing by projection. It is frequently desirable, however, to intensify the silver halide image, e.g., by reducing it to a metallic silver image, by toning it with sodium sulfide, sodium selenide, etc. or by converting it to a dye image, e.g., by reacting it with a primary aromatic amine color developing agent in the presence of a color coupling compound either in the developing bath or previously present in the emulsion. Reduction to a metallic silver image is a particularly preferred process for intensification and in such a process the elements of this invention are especially advantageous. With elements like those disclosed in Blake, U.S. Patent 3,155,519, reduction of the silver image can be effected with a conventional photographic developing agent, e.g., hydroquinone or N-methyl-p-aminophenol. Before reduction, however, it is customary to fog the emulsion by an overall flash exposure to white light. The elements of the present invention have the advantage that they do not require a flash exposure step. This elimination of such a step is quite significant and simplifies processing. Moreover, flashing is impractical and undesirable in darkrooms where multiple processing operations may be carried on simultaneously.

Suitable organic compounds which may be used to form silver salts in intimate association with the silver halide crystals include those azole compounds coming

within the scope of the above-designated Formula I. The utility or any such azole compound can be readily determined by relatively simple tests. Essentially, the utility is determined by Test A and Test B. In Test A, the candidate azole compound must render a dispersion of silver halide crystals insoluble in a silver halide solvent, e.g., an aqueous solution of sodium thiosulfate, at some pH between 1 and 13. If the candidate compound meets the insolubility requirements of Test A, it must also meet the requirements of Test B by forming with said dispersion of silver halide crystals a reaction product which, upon treatment with an aqueous solution of sodium hypochlorite, becomes soluble when subsequently treated with aqueous sodium thiosulfate. The following practical tests are provided in further exemplification of the invention and include specific concentrations of solutions, times, etc., so that suitable azole compounds may be readily and positively identified.

#### Test A

20 A solution nearly saturated at 25° C. with a candidate azole compound is prepared using ethanol, acetone, dimethylformamide, water or other suitable solvents. Depending on the solubility, a solution concentration from 0.01 to 10 percent by weight is obtained. Twenty-five ml. 25 of a gelatino-silver chlorobromide dispersion containing 25 mg. of silver halide (calculated as silver bromide), prepared as described below, is treated with small increments (i.e., about 0.1 to 0.2 ml. at a time) of the said candidate solution under safelight conditions (Wratten 1A filter or equivalent) until the silver halide dispersion either is rendered insoluble in 10% aqueous sodium thiosulfate or the candidate is found not to cause insolubilization. Generally insolubilization will occur upon the addition of 0.05 g. or less of said candidate compound, calculated as the pure compound. Compounds which must be used in substantially greater quantities than this, e.g., 1-2 g. to effect insolubilization are considered less preferred compounds. The silver halide dispersion insolubility is determined by taking a 0.5-ml. portion of the silver halide dispersion (after each incremental addition of the candidate azole compound), adding about 0.1 to 0.2 ml. of 10% aqueous sodium thiosulfate solution and observing the turbidity after 30 seconds.

45 As a control, there is used 25 ml. of water to which small increments of the candidate solution are added. Half-milliliter portions of the control are treated in the same manner with the sodium thiosulfate solution. The presence of visual turbidity relative to the control solution is sufficient to satisfy the definition of insolubility in this 50 test.

55 This test may be repeated for various pH increments from 1 to 13. Although there is some optimum pH value at which the test is most sensitive, this is not a sharp maximum which must be precisely attained. Rather, it has been found that there is a fairly broad range of pH values (e.g., 2.0 to 3.0 pH units) over which the test has a satisfactory sensitivity. In practice, the silver halide dispersion might be tested without adjustment (e.g., at pH 5.0 to 7.0) and if insolubilization occurs here, Test A is completed. If there is no insolubilization, the test is repeated at a higher pH (e.g., from pH 10-13). If there is still no insolubilization, the test is conducted with emulsion adjusted to a lower pH (e.g., about pH 1-3). Thus three different pH values represents a practical maximum number which must be investigated to determine whether or not insolubilization will occur.

#### Test B

70 The azole compound capable of insolubilizing a silver halide dispersion according to Test A is now ready for the next test, which again will be conducted under safelight conditions. To the above silver halide dispersion, there is added the minimum amount of a solution of the candidate azole compound found necessary for insolubilization. Half-milliliter samples of the dispersion (con-

taining 0.5 mg. AgBr or 0.29 mg. Ag) are placed in two test tubes. To one sample is added 0.5 ml. of water; to the other is added 0.5 ml. of a 5% by weight aqueous solution of sodium hypochlorite (containing 25 mg. sodium hypochlorite). Next, there is added to both samples, 1.0 ml. of an aqueous 10% by weight solution of sodium thiosulfate (containing 100 mg. sodium thiosulfate). If, after standing for up to thirty seconds, the sample treated with sodium hypochlorite clarifies (or becomes less turbid) relative to the control sample, the candidate azole compound meets the requirements of Test B and it is satisfactory for use as disclosed in this invention.

The silver halide dispersion disclosed in Tests A and B above was a lithographic emulsion having a silver halide composition of 30 mole percent AgBr and 70 mole percent AgCl. The emulsion had 20 grams of gelatin present per mole of silver halide for the steps of precipitation and ripening and was freed of unwanted, soluble, by-product salts by a coagulation and wash procedure as taught in U.S. Patent 2,489,341, wherein the silver halide and most of the gelatin were coagulated by an anionic wetting agent, sodium lauryl sulfate, using an acid coagulation environment. After washing, the emulsion coagulate was redispersed in water and without the use of additional bulking gelatin, maintaining a pH of  $6.0 \pm 0.1$  while stirring 10 min. at 110° F. Usually about 10 g. of gelatin is lost during washing, and the resulting emulsion contains about 10 g. of gelatin per mole of silver halide.

The amount of the silver azole salt present in the photographic silver halide layer should be sufficient to protect the silver halide crystals so that the unexposed crystals cannot be fixed by conventional fixing conditions, i.e., at normal times, temperatures and concentrations of silver halide solvents.

The gelatin/silver halide ratio is quite flexible and may vary from 3:1 to 1:20 depending on the particular azole compound and intended use for the emulsion layer. The imagewise solution of the exposed silver halide/azole compound stratum may be effected by the silver halide solvents commonly used as photographic fixing agents, e.g., sodium thiosulfate, alkali metal thiocyanate (e.g., sodium, potassium), concentrated solutions of potassium bromide, etc.

In intensifying the resulting silver salt image, reduction of the treated, residual silver halide may be accomplished by use of any chemical reducing agent capable of reducing silver ion to silver metal, e.g., hydroquinone, metol, sodium hydrosulfite and stannous chloride. The function of the reducing agent may be enhanced by modifying the surface properties of the treated, residual silver halide crystals by means of alcohol, thiourea, potassium iodide, etc.

The photographic compositions of this invention are pre-fogged, i.e., fogged prior to the imagewise exposure, in any convenient manner. The fogging may be carried out at any stage of manufacture. Chemical fogging can be achieved during the manufacture of the emulsion by admixing such chemicals as formaldehyde, formaldehyde-yielding compounds, stannous salts such as stannous chloride, etc.

Fogging by exposure to radiation may be accomplished with any radiation which is actinic for the particular photographic emulsion, e.g., short wave length visible light such as blue or violet, ultraviolet radiation, X-radiation, gamma radiation, etc. The time and exposure intensity are not particularly critical since the treatment is effective over a wide exposure latitude. The chemical-fogging or light-fogging treatments must cause the spontaneous reduction of at least 25% of the silver halide to silver when non-image exposed dry coatings of the silver halide are processed according to "Sequence c" of Example V.

In place of part of the gelatin, other natural or synthetic water-permeable organic colloid binding agents can be used and in some cases such binders can be used alone. Such agents include water-permeable or water-

soluble polyvinyl alcohol and its derivatives, e.g., partially hydrolyzed polyvinyl acetates, polyvinyl ethers and acetals containing a large number of intralinear



groups, hydrolyzed interpolymers of vinyl acetate and unsaturated addition polymerizable compounds such as maleic anhydride, acrylic and methacrylic acid esters and styrene. Suitable compounds of the last-mentioned type were disclosed in U.S. Patents 2,276,322; 2,276,323 and 2,397,866. The useful polyvinyl acetals include polyvinyl acetaldehyde acetal, polyvinyl butyraldehyde acetal and polyvinyl sodium o-sulfobenzaldehyde acetal. Other useful colloid binding agents include the poly-N-vinylactams of Bolton U.S. Patent 2,495,918, various polysaccharides, e.g., dextran, dextrin, etc., the hydrophilic copolymers in Shacklett U.S. Patent 2,833,650, hydrophilic cellulose ethers and esters, and polymers of acrylic and methacrylic esters and amides. Also, it has been found practical to apply silver halide layers on a base material in the essential absence of a binder, e.g., by chemical or vacuum deposition.

The emulsion may optionally contain any of the usual adjuvants customarily employed in silver halide systems as long as they do not interfere with the insolubilizing action of the essential ingredient (the silver salt of the azole compound) of the invention.

The emulsions can be coated on any suitable support, e.g., cellulose esters, cellulose mixed esters; superpolymers, e.g., poly(vinyl chloride *co* vinyl acetate), polyvinyl acetals, butyral; polystyrene; polyamides, e.g., polyhexamethylene adipamide, polyesters, e.g., polycarbonates, polyethylene terphthalate, polyethylene terephthalate/isophthalate, esters formed by condensing terephthalic acid and its derivatives, e.g., dimethyl terephthalate with propylene glycol, diethylene glycol, tetramethylene glycol, cyclohexane-1,4-dimethanol (hexahydro-p-xylene dialcohol); paper, metal, glass, etc.

The desirable concentration of the azole compound which forms the required silver salt depends on many factors such as the solubility of the azole compound, the nature of its reaction with silver halide, the size and nature of the silver halide crystals, the presence of other materials which may react with or be absorbed to the surface of the silver halide, etc. Calculations given in Blake U.S. Patent 3,155,519 show that a useful concentration of the azole compound is approximately that which can be theoretically determined as required to cover the silver halide surface with a so-called monomolecular layer. As shown in the examples below, elements suitable according to this invention can be prepared by bathing a photographic film in a solution of an appropriate azole compound. In this embodiment, the silver halide crystals near the surface of the coated emulsion stratum are in contact with a higher concentration of the azole compound. Crystals farther from the surface, are treated with less of the azole compound and, if the rate of diffusion is sufficiently slow, there may be considerably less of the azole compound (even approaching zero) reacting with the lower than with the surface silver halide crystals. In such elements, satisfactory results might be obtained with only a fraction, e.g., one-half, of the amount of the azole compound theoretically calculated as required to just cover the surface of a mole of the silver halide crystals.

With regard to Tests A and B, by reference to the above text or by calculation, it can be determined readily that the organic compound should be present in such an amount, in terms of the ratio of its weight to the surface area of said silver halide crystals, that when admixed in such ratio with an aqueous silver chlorobromide (70/30 mole percent) gelatin emulsion containing 10 g. of gelatin per mole of Ag and 0.57 mg. of Ag/ml., and said silver chlorobromide dispersion is treated with 10%, by weight, aqueous sodium thiosulfate (so that the resulting mixture

contains 0.29 mg. of silver and 100 mg. of sodium thiosulfate), at least three times the amount of silver chlorobromide remains undissolved as compared with a similar dispersion successively treated with 5%, by weight, aqueous sodium hypochlorite and 10%, by weight, aqueous sodium thiosulfate (so that the resulting mixture contains 0.29 mg. of silver, 25 mg. of sodium hypochlorite and 100 mg. of sodium thiosulfate), after vigorous agitation of the dispersion for 30 seconds at 25° C.

The invention is useful with silver halide layers free from or containing a water-permeable colloid binding agent. In a preferred embodiment of the invention pre-fogging and azole compound treatment of the silver halide is such that the resulting photosoluble element can not be exposed and developed conventionally to a practical negative silver image due to high fog.

The invention will be further illustrated by but is not intended to be limited to the following examples:

*Example I.*—An aqueous light-sensitive gelatino-silver halide emulsion containing chrome alum as a hardening agent and having a gelatin to silver halide weight ratio of 1:19 (calculated as AgBr) and with a silver halide composition of 70 mole percent chloride and 30 mole percent bromide, was applied at a coating weight of 116 mg./dm.<sup>2</sup>, calculated as silver bromide, on a vinylidene chloride copolymer subbed film base prepared as described in Example IV of Alles U.S. Patent 2,779,684. A sample of this coating was treated for 15 sec. with a solution of 0.25 gram of 2-mercapto-4-phenyl-thiazole, hereinafter referred to as "MPT," in 458 ml. of solution (solvent consisting of 269 ml. of 95 percent ethanol, 25 ml. acetone, 175 ml. water) and air dried. The dried sample was prefogged by a uniform exposure for 5 sec. to a 500-watt reflector (No. 2) floodlamp (having a maximum beam candle power of 50,000 at 10 feet with a mean color temperature of 3400° K.) placed about 6 inches above the sample, then treated with the MPT solution again for 15 seconds and dried as before. Following this, the sample was sensitometrically exposed through a conventional square-root-of-two step wedge, and a Wratten #16 filter (a yellow filter which transmits less than 1% of light below a wave length of about 510 millimicrons) by a contact printer containing 7 tungsten-filament, 100-watt incandescent bulbs at about 6 inches distance for a total of 4 minutes. The exposed sample was processed for 1 minute in a hardening fixer of pH about 4.7 to 4.8 containing 77 g. of sodium thiosulfate and 10 g. of potassium acetate per liter of solution. The treatment in the fixing solution removed a portion of the exposed silver halide leaving a positive silver halide image in the unexposed areas. This image was washed in water for 30 seconds, then exposed for 5 seconds to the 500-watt reflector photoflood lamp used for the prefogging exposure at a distance of about 6 inches to completely fog the emulsion. The sample was then treated in a high pH developer of the following composition, washed, and dried in the air:

#### DEVELOPER COMPOSITION

|                                           |     |     |    |
|-------------------------------------------|-----|-----|----|
| H <sub>2</sub> O                          | ml. | 800 | 60 |
| Na <sub>2</sub> SO <sub>3</sub> (anhdyd.) | g.  | 80  |    |
| Hydroquinone                              | g.  | 16  |    |
| 1-phenyl-4-methyl-3-pyrazolidone          | g.  | 1   |    |
| Boric acid                                | g.  | 5.5 |    |
| KBr                                       | g.  | 2   |    |
| NaOH                                      | g.  | 24  |    |
| KI                                        | g.  | 2.5 |    |
| H <sub>2</sub> O to make 1 liter.         |     |     |    |

The positive silver halide image was thus intensified by being reduced to a metallic silver image, demonstrating that an image can be formed by exposure through the yellow Wratten #16 filter.

A control sample was treated as just described above, except that the pre-fogging exposure (and first treatment

with MPT solution) were omitted. The control sample showed no positive image visible to the eye (even after intensification) corresponding to the exposure through the Wratten #16 filter. Thus it was seen that a pre-fogging exposure effects a definite extension of sensitivity to the longer wavelength portions of the visible spectrum.

*Example II.*—The following compounds were procured:

- (1) 2-mercapto-4-phenylthiazole
- (2) 2-mercapto-4-cyclohexylthiazole
- (3) 2-mercapto-4-(p-methoxyphenyl)thiazole
- (4) 2-mercapto-4-phenyloxazole
- (5) 2-mercapto-4,5-diphenylimidazole
- (6) 2-mercapto-4,5-di(p-methoxyphenyl) oxazole
- (7) 2-mercapto-4-amylthiazole.

A gelatino-silver halide emulsion coating as described in Example I was cut into a number of 6-inch by 35-millimeter strips. Half of the length of each strip was covered by a mask while the other half was white light fogged by a single flash from a high-intensity xenon flash tube strobe lamp "Ascorlight" operating at its high intensity setting (to give about a  $\frac{1}{1000}$  second exposure at a distance of 1 foot).

Seven solutions were prepared, each containing 50 mg. of one of the mercaptans listed above, dissolved in a mixture of 75 ml. ethanol and 25 ml. water. Seven film strips, half-fogged as described above, were each soaked in one of the seven solutions for 30 seconds at 68° F. Each strip was then drained, air dried in an oven at 110° F., and given a square-root-of-two step wedge exposure (across both the fogged and unfogged areas of the strip) for 1 minute using the floodlamp of Example I at 115 volts at a distance of 1 foot.

The exposed strips were processed at 68° F., first for 1 minute in an aqueous solution containing 127 g. of anhydrous sodium thiosulfate per liter to remove the photosolubilized silver halide. After washing in water for 1 minute, the strips were placed for 2 minute in a photographic developer solution (Developer A of Example V), washed 5 minutes in water and air dried at 110° F., all work being carried out under red safelights. Optical transmission densities of the strips were read and below are recorded the densities where there was no imagewise exposure ( $D_{max}$ ) and the density at Step #21 where there was maximum exposure, these densities being recorded for both the fogged and the unfogged areas of the film strips.

#### OPTICAL DENSITIES

|               | Unfogged                   |         | Fogged                     |         |
|---------------|----------------------------|---------|----------------------------|---------|
|               | Unexposed<br>( $D_{max}$ ) | Exposed | Unexposed<br>( $D_{max}$ ) | Exposed |
| Compound No.: |                            |         |                            |         |
| 1             | 0.84                       | 0.10    | 4.0+                       | 0.10    |
| 2             | 0.25                       | 0.06    | 0.90                       | 0.06    |
| 3             | 1.00                       | 0.09    | 4.0+                       | 0.09    |
| 4             | 0.47                       | 0.33    | 1.70                       | 0.35    |
| 5             | 0.21                       | 0.07    | 0.41                       | 0.07    |
| 6             | 0.25                       | 0.08    | 0.74                       | 0.08    |
| 7             | 0.39                       | 0.47    | 1.88                       | 0.80    |

Photographic elements made photosoluble by treatment with each of the above seven mercaptan compounds have thus been prefogged, i.e., the silver halide not removed by treatment with sodium thiosulfate was spontaneously developable (under safelight conditions) so as to have much higher  $D_{max}$  values than found when the prefogging treatment was omitted.

*Example III.*—A gelatin-silver chloride emulsion was digested in the presence of 1.85 grams formaldehyde per mole of silver chloride at 130° F. for 40 minutes, and later digested for 20 minutes at 160° F. in the presence of 0.53 gram of 2-mercapto-4-phenylthiazole per mole of silver chloride. As a final addition, 0.006 mole of KBr per mole of AgCl was added to the emulsion. The emulsion was coated on a vinylidene chloride copolymer

subbed polyester base as described in Example I at a coating weight of 66 mg./dm.<sup>2</sup> in terms of AgCl. The dried element was exposed sensitometrically through a Wratten #58 filter (a green filter which transmits less than 1% of light below a wave length of about 480 millimicrons) to a 500-watt reflector type photoflood at a distance of about 6 inches for 4 successive 5-second exposures. The exposed element was processed in a sodium thiosulfate hardening fixer of pH about 4.7 to 4.8 for 1 minute, washed for one-half minute, then exposed for 5 seconds to a 500-watt reflector type photoflood lamp as described in Example I at a distance of about 6 inches to completely fog the emulsion. The element was next treated for 1 minute in the high pH photographic developer solution described in Example I, then washed and dried. The resulting sample showed a slight decrease in transmission density in the region exposed to the Wratten #58 filter compared with the density obtained in an adjacent unexposed region.

A control coated element similar to the one just described, except that the emulsion digestion at 130° F. was done without formaldehyde, and the coating weight was 63 mg./dm.<sup>2</sup> in terms of AgCl, was exposed and processed in the same way as the previous element. The control exposure showed no difference in density visible to the eye between the region exposed through the Wratten #58 filter, and an adjacent unexposed region.

This example demonstrates the extension of spectral sensitivity by chemical treatment (pre-fogging) with formaldehyde.

*Example IV.*—A gelatino-silver bromochloride photographic emulsion was precipitated, ripened, washed and redispersed like the emulsion used in Tests A and B. Per mole of silver halide in the emulsion there was added a 1% by weight ethanol solution containing 0.4 g. of MPT (2-mercapto-4-phenylthiazole) and the emulsion was spectrally sensitized with an acetone solution containing 0.025 g. of a merocyanine dye of the structure:



The emulsion was stirred for 20 minutes at 160° F., cooled to 95° F., the usual coating adjuvants added, and the emulsion was coated on the film base described in Example I to a coating weight of 50 mg./dm.<sup>2</sup> of silver.

A number of samples of this coating were given an image exposure through a 20-step square-root-of-two photographic step wedge for 10 seconds at a distance of 2 feet from a No. 2 photoflood lamp (as used in Example I) operating at 115 volts. Five of these samples were given uniform preflash exposures (i.e., exposures without a step wedge, prior to the image exposures) with the same light source and distance as for the image exposures but at varying times and voltages as indicated in the table below. A sixth sample received a preflash exposure (a single flash reflected from the ceiling) from a strobe light (Heiland "Strobonar" 64-B strobe flash gun). Three samples received only the image exposure. Two samples received a uniform post flash exposure of 5 seconds at 115 volts at a distance of 15 inches with the same light source as used for the image exposures.

After the preflash and image exposures (but prior to the post flash exposures) all of the film samples were processed for 45 seconds and at 68° F. in the hardening fixer described in Example I and washed in water for 30 seconds. At this point, the last two samples only were given the post flash exposure described above. Then all of the silver halide images remaining were intensified by reduction to metallic silver by treatment for 1 minute in the high photographic developer described in Example I. The samples were washed and dried and the optical

densities given in the table below were determined using a densitometer (Western Electric RA-1100-C) with a visual yellow filter.

|    | Sample No. | Preflash exposure   | Postflash exposure     | Optical densities of areas receiving no image exposure |
|----|------------|---------------------|------------------------|--------------------------------------------------------|
| 10 | 1          | 0.5 sec., 50 volts  |                        | 2.86                                                   |
|    | 2          | 5 sec., 30 volts    |                        | 2.99                                                   |
|    | 3          | 10 sec., 30 volts   |                        | 2.95                                                   |
|    | 4          | 40 sec., 30 volts   |                        | 2.85                                                   |
|    | 5          | 80 sec., 30 volts   |                        | 2.50                                                   |
|    | 6          | Bounce Strobo Light |                        | 3.15                                                   |
|    | 7          |                     |                        | 0.62                                                   |
|    | 8          |                     | 5 sec., 115 v., 15 in. | 3.29                                                   |
|    | 9          |                     | do                     | 3.27                                                   |

The photographic developer used to intensify the image contained 2.5 g. KI per liter and was able to fog the image sufficiently to partially reduce the silver halide image in the absence of any exposure to light as seen in the data for Sample 7. However, it had been found necessary in practice, prior to this invention, to give a postflash exposure (as the Samples 8 and 9) in order to reduce substantially all of the silver halide to metallic silver. Obviously, much of the silver halide was not reduced in the absence of the postflash exposure (compare the low density of Sample 7 with the much higher densities of Samples 8 and 9).

30 Samples 1 through 6 (preflash but no postflash exposure) have good optical densities after intensification. With optimum amount of preflashing, the optical densities generally will be found to be no more than 1 to 5% below those found when postflashing is used. Pre-35 flashing has an actual sensitometric advantage in that the sensitivity to light is increased by about 20 to 40% over the sensitivity when using the postflashing technique. A more important practical advantage, however, resides in the fact that the image-exposed film can be processed 40 completely under darkroom conditions with the absence of any annoying flashing procedures which could interfere with other processing operations going on in the same room. For a commercial product, the photographic film element would logically be fogged, according to the 45 teachings of this invention, at the time of manufacture. Thus the processor can avoid the extra, and sometimes very undesirable, step of postflashing.

*Example V.*—This example further demonstrates the nature of the film elements of this invention which are 50 pre-fogged so as to have "spontaneously developable" silver halide crystals. A practical limit for the pre-fogging is that a minimum of 25% by weight of the crystals must be developable (i.e., reduced to metallic silver) 55 in the absence of other treatment by radiation or chemicals when given a "Fix and Wash" (as defined below) and then developed for 3 minutes at 68° F. with conventional agitation in a specified photographic developer solution, i.e., a solution of the following composition:

|                                          | DEVELOPER A | G.   |
|------------------------------------------|-------------|------|
| p-Methylaminophenol hydrogen sulfate     | -----       | 3.0  |
| Hydroquinone                             | -----       | 9.0  |
| Na <sub>2</sub> SO <sub>3</sub> , anhyd. | -----       | 50.0 |
| K <sub>2</sub> CO <sub>3</sub>           | -----       | 50.0 |
| KBr                                      | -----       | 4.5  |
| KI                                       | -----       | 2.0  |
| Water up to 1 liter.                     |             |      |

and given a "Final Fix" as defined below.

To demonstrate further the nature of the invention, another developer was used under the same conditions of time, temperature and agitation. This developer, designated as Developer B, was identical to Developer A except for omission of potassium iodide. Developer A is 75 capable of developing both surface and internal latent

images while Developer B is primarily effective in developing surface latent images.

Two types of "pre-fogging" exposures were used:

Type I (to form primarily a surface latent image) was a low intensity light fogging with a No. 2 reflector photoflood lamp at a distance of 2 feet for 5 seconds at 30 volts.

Type II (to form both surface and internal latent images) was a high intensity light fogging consisting of 1 flash from an electronic flash tube (Heiland "Stronobar" 64-B) placed on the test table next to test sample with light directed to reflect from a white ceiling 65 inches above the table top.

Flash designates an exposure applied later (after image solubilization) using a No. 2 reflector photoflood at 15 inches for 5 seconds at 120 volts.

Fix and wash designates a 1-minute treatment at 68° F. in an aqueous solution of sodium thiosulfate, 10% by weight, followed by a half-minute wash in water at 68° F.

Final fix designates a 5-minute treatment at 68° F. in the hardening acid fixer of Example I followed by a 10 minute water wash at 68° F. and drying of the sample in air. This final fix while not used in the regular image-forming photosolubilization process, adds to an understanding of the process by removing any final, residual silver halide which is not reduced to metallic silver by one of the developer solutions. Thus the readings of silver in mg./dm.<sup>2</sup> at the end of processing, which are obtained by X-ray fluorescence, will show only developed silver.

A number of film samples were taken from a coating like that described in Example IV except that the coating weight was 104 mg./dm.<sup>2</sup> of silver halide, calculated as AgBr. These samples were given a light-fogging exposure of Type I or Type II and then processed according to one of the sequences a, b, c, d or e as indicated in the table below. The optical transmission densities (D) of the processed strips were determined as in Example IV. The silver content, Ag, was determined in units of mg./dm.<sup>2</sup> by means of X-ray fluorescence. Several samples of the coating were found, in the absence of any processing, to have an average silver content, Ag, of 61.6 mg./dm.<sup>2</sup>.

5

10

15

20

25

30

35

40

45

containing Developer A, which is the sequence of normal photosolubilization processing (fixing to form a positive image and then intensifying), it is seen that in the absence of prefogging there is virtually no developed silver while Type I and Type II prefogging treatments give, respectively, 17.1 and 17.2 mg./dm.<sup>2</sup> silver contents. Since the unprocessed coatings had silver contents of 61.6 mg./dm.<sup>2</sup>, these values mean that 27.7% and 27.9%, respectively, of the total weight of the silver halide was spontaneously developable.

The requirement that these values exceed 25% provides practical limits for the required extent of the pre-fogging treatment. With insufficient pre-fogging, less than 25% of the silver halide can be reduced to metallic silver. Also, it is obvious that excess pre-fogging by light will photosolubilize the silver halide causing loss via solubilization during the "Fix & Wash" part of Sequence c to the extent that less than 25% of the silver halide remains for conversion to metallic silver.

Whereas Sequence c represents the normal photosolubilization processing of areas of an element receiving no imagewise exposure, Sequence a represents the corresponding process in areas receiving full imagewise exposure. Less than 1% of the silver halide has been developed to metallic silver in such fully exposed areas since the first step of the processing sequence (fixing) has removed the photosolubilized silver halide before it could be developed. Therefore, Sequences a and c taken together demonstrate that the pre-fogged photosolubilizable film element is capable of giving a positive silver halide image which can be intensified in a photographic developer without immediate prior flashing with light.

The prefogging exposure and other conditions are not fully optimized in this example as can be seen by comparing Sequences b and c. Although Sequence c shows that over 25% of the silver halide is spontaneously developable, the extra flashing step of Sequence b (prior to the development step) brings the total developed silver up to about 35% of that originally in the element.

Sequences d and e, taken together, show that the element, with either Type I or Type II prefogging, is not suitable for conventional processing (wherein development precedes fixing) to give a negative image. It is obvious that there is insufficient difference in the amount of

|                       | Processing sequence |            |            |       |            |       |                  |       |
|-----------------------|---------------------|------------|------------|-------|------------|-------|------------------|-------|
|                       | a                   |            | b          |       | c          |       | d                |       |
|                       | Flash               | Fix & Wash | Fix & Wash | Flash | Fix & Wash | Flash | Fix & Wash       | Flash |
| Developer A Final Fix |                     |            |            |       |            |       |                  |       |
| Light fogging-----    | D                   | Ag         | D          | Ag    | D          | Ag    | D                | Ag    |
| None-----             | .03                 | 0.4        | 3.10       | 21.8  | 0.00       | 0.2   | 3.68             | 28.3  |
| Type I-----           | .05                 | 0.4        | 3.18       | 21.3  | 2.20       | 17.1  | 4.0 <sup>+</sup> | 32.5  |
| Type II-----          | .03                 | 0.3        | 3.20       | 22.0  | 2.20       | 17.2  | 3.80             | 28.3  |

The above processing was carried out on other samples of the coating except that Developer A was replaced with

developed silver and in the optical transmission densities between areas receiving full imaging exposure (Se-

|                                     | Processing sequence |            |            |       |            |       |                  |       |
|-------------------------------------|---------------------|------------|------------|-------|------------|-------|------------------|-------|
|                                     | a                   |            | b          |       | c          |       | d                |       |
|                                     | Flash               | Fix & Wash | Fix & Wash | Flash | Fix & Wash | Flash | Fix & Wash       | Flash |
| Developer B (which contained no KI) |                     |            |            |       |            |       |                  |       |
| None-----                           | .03                 | 0.2        | 3.30       | 23.8  | 0.01       | 0.6   | 4.0 <sup>+</sup> | 32.7  |
| Type I-----                         | .03                 | 0.5        | 3.74       | 26.7  | 0.90       | 8.3   | 4.0 <sup>+</sup> | 35.4  |
| Type II-----                        | .03                 | 1.1        | 3.60       | 25.2  | 0.41       | 4.2   | 4.0 <sup>+</sup> | 32.1  |

The following information obtained from the table is of significance to this invention.

First, the photosolubilizable elements of this invention require "pre-fogging" to the extent that at least 25% by weight of the silver halide crystals must be spontaneously developable by the prescribed treatment in Developer A. Referring to processing Sequence c with potassium iodide-

70 sequence d) and areas receiving no imaging exposure (Sequence e). Thus the densities recorded in Sequence e represent undesirably high fog densities.

The second set of processing data involving the use of Developer B (without potassium iodide) are included for the sake of completeness but merit less discussion. With 75 prefogging by means of light, there is sufficient internal

fogging of the crystals that it is definitely preferred to employ a developer such as Developer A which is capable of reducing both surface and internally fogged crystals.

*Example VI.*—Chemical pre-fogging has been found to be more efficient than prefogging by light and, among the chemical agents used, formaldehyde or formaldehyde-yielding compounds are particularly preferred. One mole of a gelatin-silver chloride emulsion, containing 105 g. of gelatin, was digested for 40 minutes at 130° F. in the presence of 1.87 g. of formaldehyde. Later it was further digested 20 minutes at 170° F. in the presence of 0.76 g. of 2-mercapto-4-phenylthiazole and 0.025 g. of the optical sensitizing dye of Example IV. The emulsion was coated on the film base of Example I at a coating weight of 58 mg./dm.<sup>2</sup> of silver chloride. A control coating was prepared in a similar manner but no formaldehyde was present to effect pre-fogging.

Samples from the two coatings were processed according to the 5 processing sequences described in Example V, using Developer B (containing no potassium iodide) for intensification.

The results are shown below:

OPTICAL TRANSMISSION DENSITIES

| 5                                         | Processing sequence   |                       |                      |
|-------------------------------------------|-----------------------|-----------------------|----------------------|
|                                           | a                     | b                     | c                    |
|                                           | Flash<br>Fix and Wash | Fix and Wash<br>Flash | xxxx<br>Fix and Wash |
| Developer A Final Fix                     |                       |                       |                      |
| Prefogging.....                           |                       |                       |                      |
| None.....                                 | 0.0                   | 1.67                  | .20                  |
| SnCl <sub>2</sub> ·2H <sub>2</sub> O..... | 0.04                  | 1.90                  | 1.94                 |

The composition and elements of this invention have all of the utility and advantages disclosed in assignee's applications that are listed above. Thus, the photographic processes applicable to the new products of the invention can be used to form a useful positive silver halide image in only a single step following the exposure. This image may be intensified to a metallic silver image by a process of total reduction since the non-image silver halide has already been removed. This total reduction is a simpler

|                       | Processing sequence |                     |                    |               |              |
|-----------------------|---------------------|---------------------|--------------------|---------------|--------------|
|                       | a                   | b                   | c                  | d             | e            |
|                       | Flash<br>Fix & Wash | Fix & Wash<br>Flash | xxxx<br>Fix & Wash | xxxx<br>Flash | xxxx<br>xxxx |
| Developer B Final Fix |                     |                     |                    |               |              |
| Prefogging.....       | D                   | Ag                  | D                  | Ag            | D            |
| None.....             | 0.0                 | 0.3                 | 3.12               | 14.6          | 0.0          |
| Formaldehyde.....     | 0.0                 | 0.2                 | 3.75               | 19.1          | 3.20         |
|                       |                     |                     |                    |               | 15.7         |

For unprocessed samples of the two coatings, the average silver content, Ag, was 39.2 mg./dm.<sup>2</sup>.

When the above data are carefully considered and compared with Example V, the same general conclusions can be reached. In normal photosolubilization processing Sequence c the prefogged silver halide is calculated to be 40% spontaneously developable

$$\left( \frac{15.7 \times 100}{39.2} = 40\% \right)$$

while there is almost no spontaneous development in the non-prefogged coating.

Very similar results are obtainable when Developer A (containing potassium iodide) is substituted for Developer B.

*Example VII.*—Chemical prefogging was effected by stannous chloride as follows: One mole of a gelatin-silver chloride emulsion, containing 101 g. of gelatin, was digested for 40 minutes at 130° F. in the presence of 0.07 g. of SnCl<sub>2</sub>·2H<sub>2</sub>O. Later it was further digested 20 minutes at 170° F. in the presence of 0.75 g. of 2-mercapto-4-phenylthiazole and 0.025 g. of the optical sensitizing dye of Example IV. The emulsion was coated on the film base of Example I at a coating weight of 52 mg./dm.<sup>2</sup> of silver chloride. A control was prepared in a similar manner but no stannous chloride was present to effect pre-fogging.

Samples from the two coatings were processed according to processing Sequences a, b and c described in Example V, but using the following developer formulation for intensification.

|                                                |    |         |
|------------------------------------------------|----|---------|
| Water -----                                    | ml | 800     |
| Na <sub>2</sub> SO <sub>3</sub> (anhyd.) ----- | g  | 80      |
| Hydroquinone -----                             | g  | 16      |
| 1-phenyl-4-methyl-3-pyrazolidone -----         | g  | 1       |
| Boric acid -----                               | g  | 5.5     |
| NaOH -----                                     | g  | 16      |
| 0.5 M KI -----                                 | ml | 30      |
| Water to make 1 liter.                         |    |         |
| pH at 68° F. -----                             |    | 12.5 75 |

35 reaction than the selective reduction required in conventional photographic processing where it is necessary to reduce only that silver halide which has been exposed to light.

*Example VIII.*—A photographic layer was made by evaporating silver chloride onto the film base described in Example I, using a High Vacuum Evaporator, Model No. SC-3 (Optical Film Engineering Co.). The vacuum apparatus employed a tantalum ribbon and operated at a pressure of  $3 \times 10^{-4}$  microns of mercury. Using about 280 milligrams of AgCl at a distance of 24 cm. from the film base, a coating weight of AgCl of about 4 mg./dm.<sup>2</sup> was obtained.

The vacuum-coated film was bathed for 15 sec. in the ethanol-water (25/10) solution of 2-mercapto-4-phenylthiazole of Example I, dried and exposed stepwise for 5, 10, 20, 40 and 80 seconds to a photoflood lamp (General Electric 2-A) at a distance of 6 inches. The exposed element was then immersed in 12.8% aqueous sodium thiosulfate for 30 seconds, rinsed in water for 10 seconds and then bathed in a developer solution as described in Example I. All operations were carried out under illumination from white fluorescent lamps. Such illumination during the preparation of the element and subsequent steps provided the pre-fogging required according to this invention.

60 A direct-positive image was formed by the 5, 10, 20 and 40-second exposure, i.e., imagewise density decreased with increasing exposure. However, when the exposure was increased to 80 seconds, a negative image was formed, the system reversing or solarizing by increased exposure like conventional silver halide systems.

An important advantage of the novel elements of this invention over those of the listed applications is their enhanced spectral sensitivity. These elements can be exposed by light of various wavelength and can, therefore, produce more faithful recordings of original scenes. A very practical advantage is shown in connection with Example IV wherein it is demonstrated that prefogging (which could be carried out during manufacture of the film) could eliminate post-flashing and any disadvantages thereof.

The most obvious advantage of the novel elements of this invention is the extension of their spectral sensitivity. These elements can be exposed by light of various colors and can, therefore, produce more faithful recordings of original scenes.

Another advantage of this invention is that it provides new elements for forming silver images that do not require special equipment but instead can be used with conventional equipment and apparatus. A further advantage is that the elements can be used successfully by photographers of ordinary skill. A still further advantage is that the elements can be processed with conventional reducing agents, e.g., developers and conventional fixing agents. Yet another advantage is that the new elements can be used to produce images without selective reduction.

The embodiments of the invention in which an exclusive property or privilege is claimed are defined as follows:

1. A photosoluble silver halide dispersion comprising, before imagewise exposure to radiation, light-sensitive silver halide crystals having associated therewith in substantially greater than fog-inhibiting amounts a silver salt of an organic compound of the formula



where X is a member selected from the group consisting of S, O and NH, R<sub>4</sub> is a hydrocarbon nucleus of 4-8 carbon atoms, and R<sub>5</sub> is hydrogen or a hydrocarbon nucleus of 4-8 carbon atoms, said salt being of lower solubility in water than silver chloride; the silver halide crystals so associated with the silver salt being less soluble in 10% aqueous sodium thiosulfate than untreated silver halide crystals at a predetermined pH and the associated silver salt being present in such an amount, in terms of the ratio of its weight to the surface area of said silver halide crystals, that when admixed in such ratio with an aqueous silver chlorobromide (70/30 mole percent) gelatin emulsion containing 10 g. of gelatin per mole Ag and 0.57 mg. of Ag per ml., and said silver chlorobromide dispersion is treated with 10%, by weight, aqueous sodium thiosulfate (so that the resulting mixture contains 0.29 mg. of silver and 100 mg. of sodium thiosulfate), at least three times the amount of silver chlorobromide remains undissolved as compared with a similar dispersion successively treated with 5%, by weight, aqueous sodium hypochlorite and 10%, by weight, aqueous sodium thiosulfate (so that the resulting mixture contains 0.29 mg. of silver, 25 mg. of sodium hypochlorite and 100 mg. of sodium thiosulfate), after vigorous and essentially equal agitation of both dispersions for 30 seconds at 25° C.; characterized in that the silver halide crystals are spontaneously developable to the extent that over 25% by weight of the silver of said crystals remains as reduced silver after dissolving, washing and development for 3 minutes at 68° F. in an aqueous developer of the following composition:

|                                        |      |       |
|----------------------------------------|------|-------|
| p-N-methylaminophenol hydrogen sulfate | 3.0  | G. 65 |
| Hydroquinone                           | 9.0  |       |
| Na <sub>2</sub> SO <sub>3</sub>        | 50.0 |       |
| K <sub>2</sub> CO <sub>3</sub>         | 50.0 |       |
| KBr                                    | 4.5  | 70    |
| KI                                     | 2.0  |       |
| Water to make 1 liter.                 |      |       |

treatment for one minute at 68° F. in a 10% aqueous solution of sodium thiosulfate, washing for one-half min-

ute with water at 68° F., treatment for 5 minutes at 68° F. in a hardening aqueous fixing solution of pH about 4.7 containing 77 g. of sodium thiosulfate and 10 g. of potassium acetate per liter of solution followed by washing in water at 68° F.

5 2. A dispersion according to claim 1 wherein said silver salt is a mercaptide of 2-mercapto-4-phenylthiazole.

3. A dispersion according to claim 1 wherein said silver salt is a mercaptide of 2-mercapto-4-cyclohexylthiazole.

10 4. A dispersion according to claim 1 wherein any heavy metal salt present is a noble metal salt.

5. A dispersion according to claim 1 wherein there is present a water-permeable organic colloid binding agent 15 for the silver halide crystals.

6. A photographic element comprising a support comprising a layer of a photosolubilizable silver halide dispersion comprising, before imagewise exposure to radiation, light-sensitive silver halide crystals as defined in 20 claim 1.

7. An element according to claim 1 wherein said silver salt is a mercaptide of 2-mercapto-4-phenylthiazole.

8. An element according to claim 1 wherein said silver salt is a mercaptide of 2-mercapto-4-cyclohexylthiazole.

25 9. An element according to claim 1 wherein any heavy metal salt present is a noble metal salt.

10. An element according to claim 1 wherein there is present a water-permeable organic colloid binding agent for the silver halide crystals.

30 11. An element according to claim 1 wherein the layer is free from a binding agent for the silver halide crystals.

12. A process which comprises giving an overall pre-fogging exposure to a light-sensitive silver halide layer and then admixing therewith in substantially greater than 35 fog-inhibiting amounts a silver salt of an azole compound of the formula:



40 where X is a member selected from the group consisting of S, O and NH, R<sub>4</sub> is a hydrocarbon nucleus of 4-8 carbon atoms, R<sub>5</sub> is hydrogen or a hydrocarbon radical of 4-8 carbon atoms, said salt being of lower solubility in water than silver chloride; the silver halide crystals so associated with the silver salt being less soluble in 10% aqueous sodium thiosulfate than untreated silver halide crystals at a predetermined pH and the associated salt of the azole compound being present in such an amount, in terms of the ratio of its weight to the surface area of said silver halide crystals, that when admixed in such ratio with an aqueous silver chlorobromide (70/30 mole percent) gelatin emulsion containing 10 g. of gelatin per mole Ag and .57 mg. of Ag per ml., and said silver chlorobromide dispersion is treated with 10%, by weight, aqueous sodium thiosulfate (so that the resulting mixture contains 0.29 mg. of silver and 100 mg. of sodium thiosulfate), at least three times the amount of silver chlorobromide remains undissolved as compared with a similar

45 dispersion successively treated with 5%, by weight, aqueous sodium hypochlorite and 10%, by weight, aqueous sodium thiosulfate (so that the resulting mixture contains 0.29 mg. of silver, 25 mg. of sodium hypochlorite and 100 mg. of sodium thiosulfate), after vigorous and essentially equal agitation of both dispersions for 30 seconds at 25° C.

50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 87

## References Cited

## UNITED STATES PATENTS

|           |         |          |       |        |
|-----------|---------|----------|-------|--------|
| 436,587   | 9/1890  | Schwartz | ----- | 96—107 |
| 3,062,651 | 11/1962 | Hillson  | ----- | 96—95  |
| 3,155,519 | 11/1964 | Blake    | ----- | 96—64  |
| 3,253,919 | 5/1966  | Beavers  | ----- | 96—50  |

by Colloidal Silver, in Franklin Institute Journal, pp. 587—590, November 1930.

NORMAN G. TORCHIN, Primary Examiner

5 R. E. FICHTER, Assistant Examiner

U.S. Cl. X.R.

## OTHER REFERENCES

96—64

Sheppard, S. S.: The Optical Sensitizing of Silver Halides